

Aug. 26, 1947.

C. S. SMITH, JR

2,426,377

SELENIUM RECTIFIER AND METHOD OF MAKING

Filed Dec. 7, 1943

2 Sheets-Sheet 1

Fig. 1



Fig. 2



Fig. 3



Fig. 5



INVENTOR.  
CLEVELAND SCUDDER SMITH, JR.

BY

Robbin & Carlson

ATTORNEYS



Aug. 26, 1947.

C. S. SMITH, JR

2,426,377

SELENIUM RECTIFIER AND METHOD OF MAKING

Filed Dec. 7, 1943

2 Sheets-Sheet 2



INVENTOR.

CLEVELAND SCUDDER SMITH, JR.

BY

Robbin + Carlson

ATTORNEYS

## UNITED STATES PATENT OFFICE

2,426,377

SELENIUM RECTIFIER AND METHOD  
OF MAKINGCleveland Scudder Smith, Jr., Indianapolis, Ind.,  
assignor to Samuel Ruben, New Rochelle,  
N. Y.

Application December 7, 1943, Serial No. 513,265

11 Claims. (Cl. 117—107)

1

This invention relates to metal rectifiers and photocells, and to methods and apparatus for depositing a relatively thin layer or layers of a metal such as selenium upon a base composed of a different metal or alloy.

It has long been recognized that when the surfaces of certain metals or metallic compounds are placed in contact with each other such combination possesses photoelectric characteristics and is also capable of rectifying an alternating electric current. While numerous combinations of metals and metallic compounds have been proposed for use as rectifying and photoelectric elements, one of the most satisfactory combinations is a layer or film of selenium deposited upon an aluminum, bronze, copper or ferrous metal base and having a counter-electrode deposited upon or in contact with its exposed surface. However, due to its inherent chemical characteristics selenium is difficult to control and of its several known forms which exist at room temperature only one form appears to possess photoelectric and rectifying properties. To be suitable for use in a photoelectric or rectifying element, selenium must be present substantially or entirely in the form of a thin gray metallic film upon a suitable base metal. If the conditions for depositing the selenium are not carefully controlled, a useless deposit of the amorphous or crystalline form of selenium may result.

Various methods for the deposition of a layer of selenium on a base metal for the manufacture of rectifiers and photocells have been proposed. In general, such processes involve the application of selenium, either in paste or powder form, to a previously prepared base plate while the latter is maintained at an elevated temperature. Another suitably heated metal plate is then brought in contact with the paste, and the assembly is subjected to a hot pressing operation to form a structure having an inner layer of metallic selenium. This method possesses several inherent disadvantages which render it impractical for commercial use. For instance, a layer of selenium cannot easily be formed which has controlled variation in chemical or electrical characteristics throughout the body of the selenium, furthermore, several successive layers cannot readily be built up to form a homogeneous larger layer. In addition, such known process is not only costly in time required for carrying out the numerous steps, but it is impractical for the commercial manufacture of large plate rectifiers because of unavoidable variations in plate thickness, the random orientation of the resulting

crystalline deposit, and the erratic and poor rectifying characteristics of such surface.

Another process has been proposed in which the plates to be coated with selenium are passed the discharge orifices of one or more selenium boilers or are mounted at fixed distances from stationary selenium boilers, the plates and boiler or boilers being disposed in an evacuated chamber maintained at a pressure of the order of 1 micron of mercury or less. Such process is necessarily a batch process and is not adapted to the rapid and continuous production of photocell and rectifier elements. Also, because of the long pumping time required to obtain the desired vacuum, and because of practical limitations on the size of the vacuum system, such process is highly uneconomical for the manufacture of large size elements or for the deposition of more than one layer of selenium both in first cost, operating cost and maintenance cost.

The present invention overcomes the numerous disadvantages inherent in prior processes and provides a method and apparatus for the economical and commercial production of selenium photocell and rectifier elements.

Accordingly, among the objects of this invention are: to provide an improved method in which selenium is deposited on a base plate under ordinary atmospheric conditions in the form of as many different layers of metallic selenium as may be desired; to provide a method in which the selenium deposition is uniform and the thickness of such deposit may be accurately controlled to any desired value; to provide a method which is adapted to the automatic, continuous and efficient production of selenium photocell and rectifier elements; to provide apparatus of relatively simple design which is adapted to carry out the method of the invention.

40 The above and other objects, advantages and novel features of the invention will become apparent from the following description and accompanying drawings, in which:

Fig. 1 shows an elevational view, in cross-section, of one form of an apparatus embodying the principles of this invention;

Fig. 2 is an enlarged sectional view taken from the left along the line 2—2 of Fig. 1;

Fig. 3 is an elevational view, partly in cross-section, of a modification of the apparatus of the invention,

Fig. 4 is an enlarged sectional view of one of the several selenium vaporizing boilers or units illustrated generally in Fig. 3;

55 Figs. 5 and 6 are elevational views of a further

## 3

modification of the selenium vaporizing boilers or units embodying the principles of this invention:

Fig. 7 is an elevational view, partly in section of an apparatus adapted to coat a film or thin layer of selenium simultaneously on both sides of a metal plate;

Fig. 8 illustrates a method of applying a metal counter-electrode onto a metallic plate; and

Figs. 9 and 10 illustrate partially completed rectifier blanks.

In general, the improved method of this invention is carried out by vaporizing selenium in a suitable boiler above and substantially at atmospheric pressure and impinging the resulting vapor against the surface of a suitable metal plate maintained either at or above room temperature. The boiler is preferably provided, in one embodiment of the invention, with a slotted discharge orifice which has a length greater than or substantially equal to the width of the plate to be coated. The metal plate to be coated is maintained at a preselected distance from the orifice of the boiler and when such plate is moved back and forth through the stream of selenium vapor issuing from such orifice, at a preselected rate and in a direction substantially transversely of the longitudinal direction of the slot orifice, an extremely smooth and uniform film or layer of gray metallic selenium of desirable rectifier or photocell quality is deposited on the metal plate. By making several passes back and forth through the stream of vapors issuing from the orifice, any desired thickness of selenium may be built up. If desired, several boilers may be disposed in tandem relation, so that the metallic plate may pass successively through several streams of selenium and thereby quickly build-up a plurality of layers of selenium. In such an arrangement the boilers may be operated to discharge the same or different concentrations of vapors, and different impurities may be introduced into the several boilers to build up selenium of desirable composition for low forward resistance and high reverse resistance.

Referring to the drawings, Figs. 1 and 2 illustrate an embodiment of the invention wherein a selenium boiler B comprising a cylindrical casing 12 is provided with an upper threaded portion 14 adapted to frictionally engage a threaded portion 16 of a cap 18. A slotted orifice 20 is provided in cap 18, and has substantially uniform cross-section throughout its length. The orifice 20 has a length substantially equal to the inside diameter of the casing 12. A circular flange 22 is welded as at 23, or otherwise secured, to the cap 18 to support the boiler and to position the upper surface of the cap 18 substantially flush with the upper surface of a suitable supporting base board 24, which may be composed of asbestos or other non-inflammable material. Guides 26 are secured to the base board 24 along lines equidistant on either side of the boiler B. These guides 26 are adapted to support a slide 28 carrying the metal plates 30 to be coated with selenium. The metal plates 30 may be bolted at 32 or otherwise secured to the carriage 28, and co-operate with suitable grooves 34 in the guides 26. A knob or handle 128 is provided to slide the plates back and forth on the boiler. The distance between the top of the cap 18 and the surface of the metal plate to be coated with selenium, is maintained at a value such that when selenium vapor streams at the desired rate through the

## 4

slotted orifice the lower surface of the metallic plate is uniformly coated. A pair of gas burners 36 or other heating agents may be used to vaporize the selenium, and in order to prevent condensation of selenium vapor in the upper part of the boiler B, the heat is preferably applied to the upper regions of the boiler.

The method of carrying out the invention to obtain a coating of selenium upon a metal plate is as follows: Boiler casing 12 is unscrewed from cap 18, and about 10 grams or more of selenium is deposited in the boiler; the casing is then screwed back into position in the cap 18, and suitably heated as by one or more gas burners to a temperature sufficient to cause a stream of selenium vapor to issue through the orifice 20. Heat is applied to the upper portion of the boiler to avoid condensation of selenium therein and is conducted downward by the boiler walls to vaporize the selenium charge. When selenium vapor is issuing at the desired rate from the orifice, the slide or carriage 28, carrying the metal plates to be coated, is inserted in the guides and a number of passes are made back and forth through the stream of selenium vapor thereby forcing a thin adherent coating of selenium upon the surface of the plates.

It has been found that during each deposition of selenium thin films are formed on the previous surface and on the new selenium surface, which films are composed of a mixture of selenium oxides, water and condensed particles of selenium in forms unsuitable for rectifiers. These films may cause the selenium to peel or crack, and they may produce high forward resistance in the completed rectifier.

Usually the interspersed films are so thin as to cause no adverse effects on the completed rectifier. The films can be completely eliminated by conducting the deposition of selenium in an atmosphere of inert gas such as argon, a relatively inert gas such as nitrogen, or carbon dioxide, or a reducing gas such as household cooking gas. The surrounding gas may be at any desired temperature, and should be above the boiling temperature of selenium if it is desired to avoid any condensation of selenium before the selenium vapor reaches the receiving plate.

The ratio of length to width of the orifice is somewhat critical to the deposition of the desired layer of selenium. For example, an orifice width of about 0.012 inch has been found to yield good results. A smaller width gives a greater proportion of selenium oxide to selenium. Slight variations in the width of the orifice slit are to be avoided because such variations cause striations to appear in the deposited selenium. A greater orifice width makes it difficult to build up sufficient pressure in the boiler to permit uniform vapor flow along the entire length of the orifice slit, and also causes a greater quantity of selenium vapor to emerge than is necessary or desirable. Hence, care in construction and choice of materials may dictate the use of smaller orifice widths.

The distance of the plate from the discharge orifice must be carefully selected to give the most desirable results. In general, the closer the plate is brought to the orifice, the more satisfactory is the deposition of selenium. If the operation is carried out under conventional atmospheric conditions, some of the selenium oxidizes and some of the selenium condenses to fine red particles. The greater the plate dis-

tance, the greater is the ratio of oxidized and condensed selenium to selenium still in vapor form. Too large a proportion of selenium oxide and selenium condensed to the red particle form causes the selenium to peel and crack from the base plate during later heat treatment and may also lead to high resistance in the forward direction.

Other factors which influence the characteristics of the deposited selenium are: speed of the plate past the boiler orifice, rate of selenium flow and number of passes made by the plate past the orifice. All of the above factors must be correlated to give the most desirable type of selenium deposition.

The temperature of the plate or plates upon which selenium is to be deposited has not been found to be critical, but plates maintained at a temperature of between about 60° to 100° C. are satisfactory and yield a smooth black deposit of selenium, which is desirable in the manufacture of rectifier elements.

Figure 3 illustrates a modification in which a long or continuous band of metal 37 is led over a series of selenium boilers B', which may be heated in any manner, as with electric resistance heating coils 39. The boilers may all be identical in construction or may differ as to width of orifice or other factors to superimposed layers of different thickness or other characteristics. After coating, the strip may be cut into rectifier elements of the desired dimensions.

Figure 4 shows a boiler modification wherein a gaseous atmosphere is introduced by a conduit 38 into a boiler B<sup>2</sup>, the upper portion of which is heated by a high frequency inductance coil 40. The heat travels downward to vaporize the selenium but the upper part of the boiler is kept hottest to prevent condensation. The gaseous atmosphere entering through conduit 38 may comprise an inert gas such as argon, a relatively inert gas such as nitrogen or carbon dioxide, or a reducing gas. The boiler may be alternatively heated by gas, by radiant heat from an electrical heater, by conducted heat from an electric heater, by electromagnetic induction, or by other convenient means.

Figure 5 illustrates a two compartment boiler, wherein compartment 44 is adapted to receive solidified selenium or melted selenium at low temperature and compartment 46 is adapted to vaporize molten selenium flowing from compartment 44. A valve 48 is disposed in the base of the boiler to drain off the selenium or the accumulation of excessive amounts of impurities.

In the embodiment shown in Figure 6, molten heated selenium may be introduced into a boiler 50 from a vessel 51, through a needle valve 52. Sufficient heat is applied to 50 to cause the selenium to vaporize and flow through a slotted orifice 54. The amount of selenium vaporized in this type of boiler can be accurately controlled by the setting of the needle valve 52 and the pressure behind the selenium in the vessel 51. In this modification the boiler orifice 54 is shown in a position such that the vapors stream downwardly onto the metal plates to be coated, but the orifice may be arranged so that the selenium vapor emerges therefrom in any direction whatsoever.

Figure 7 illustrates a modification wherein both sides of a metal plate 56 are simultaneously coated with selenium. A vertically elongated orifice 58 of a suitable selenium boiler is disposed on either side of the plate 56 which is mounted in a

slide 60. When the selenium vapor issues at the desired rate from each orifice the plate 56 is moved past the orifices in a manner similar to that described in connection with Figure 1.

Figure 8 shows a method for applying a metal counter-electrode on top of the selenium deposit 62 on a metal plate 61. A mask 63 having apertures or windows 64 is placed against the selenium surface and a soft, low-melting-point metal 68 is sprayed onto the exposed areas of selenium by the metal spray gun 65 supplied with compressed air by air hose 66 and containing molten metal heated by an electric heating element supplied by wires 70.

Figure 9 shows a plate after spraying, comprising backing metal plate 61 with selenium coating 62, and several sprayed metal electrodes 72 on the selenium surface. This plate may be cut into individual rectifier units.

Figure 10 shows an improved plate wherein the backing plate 79 is notched at intervals before the selenium layer 78 is applied. After spraying of electrodes 72 the strip can be readily broken or cut at the notches.

The sequence of steps or operations in the production of rectifier elements according to this invention is substantially as follows:

(1) The metal strips to be coated with selenium are grooved by means of a kick press or automatic power press.

(2) They are then cleansed in any suitable manner, e. g. by immersion in a cleaning solution, a cleaning vapor, or wiping with a rag.

(3) Both sides of the metal strips are then sand-blasted, as for example, with Carborundum of a particle size of 240 to 280 mesh, the metal strips being driven between rollers at a linear speed of about 10 ft. per minute, one sand blast being directed against each side.

(4) The next step is the selenium deposition substantially as described above.

(5) The selenium plated strips are next heat treated at a temperature of about 210° C. for a period ranging from 15 minutes to one hour.

(6) A blocking layer is then applied to the plates, this consisting of a thin film of selenium oxide. This may be effected, for example, by exposing the plates to selenium oxide vapors in a closed chamber for a few seconds, or by any other suitable method.

(7) The plates are next sprayed with a metal or alloy having a melting point below the melting point of selenium.

(8) The final operation is the forming treatment, which consists in subjecting the plates to a suitable direct current, applied through contacts engaging the metal base plate and the sprayed metal layer in a direction in which the element tends to block current flow. This inverse current is applied for a period of about 2 to 6 hours, at a current density of, for example, about 300 milliamperes per sq. inch of active area.

While certain embodiments of the invention have been specifically illustrated and described, it is understood that the invention may be otherwise embodied and practiced without departing from the principles or scope of the invention as set forth in the appended claims.

What is claimed is:

1. The method of depositing a layer of selenium of substantially uniform thickness upon a metal surface which comprises the steps of vaporizing selenium at substantially atmospheric pressure, causing the resulting vapors to assume the shape of a thin ribbon, surrounding said

stream with an envelope of gas selected from the group consisting of reducing gases and inert gases, and establishing relative transverse movement between said ribbon of gas and said surface to effect the condensation and deposition of a gray, metallic layer of selenium upon said surface.

2. In the art of depositing a selenium layer of substantially uniform thickness upon at least one surface of a metal base, the improvement which comprises the steps of vaporizing selenium at substantially atmospheric pressure, forming the resulting vapors into a thin ribbon-like stream in substantially unadulterated vaporized form, surrounding said stream with an envelope of gas selected from the group consisting of reducing gases and inert gases, moving said metal base so as to intersect said stream in a direction perpendicular to the widest dimension of said stream to form a thin, uniform and adherent coating of selenium in the gray, metallic state upon said surface, and repeating said movement back and forth through said stream to form a selenium layer of desired thickness.

3. Apparatus for depositing a relatively thin layer of selenium upon a metal base comprising, in combination, means for vaporizing and forming a thin ribbonlike stream of selenium vapor substantially at atmospheric pressure, means for supporting and bringing a base into contact with said stream of selenium vapor, and means for mixing a gas selected from the group consisting of inert gases and reducing gases with said stream of selenium vapor.

4. Apparatus for depositing a relatively thin layer of selenium upon a metal base, said apparatus including a selenium vaporizer operable substantially at atmospheric pressure having a relatively narrow slot-like orifice disposed in the upper portion thereof, means for externally heating said vaporizer to generate a stream of selenium vapor and to avoid condensation of said vapor in said orifice.

5. A method of depositing a layer of selenium upon a metal base which comprises vaporizing selenium at substantially atmospheric pressure, causing the resulting vapors to assume the shape of a stream, surrounding said stream with an envelope of gas selected from the group consisting of reducing gases and inert gases, and directing said stream against a metal base to form a uniform adherent coating of gray metallic selenium thereon.

6. Apparatus for depositing a layer of selenium upon a metal base which comprises a selenium vaporizing furnace having a narrow slot-like discharge orifice, means for applying heat to said furnace adjacent said discharge orifice to prevent condensation of selenium vapors in the regions near said orifice, and a guide for supporting a metal base a preselected distance from said orifice.

7. Apparatus for depositing a layer of selenium upon a metal base which comprises a selenium vaporizing furnace having a narrow slot-like discharge orifice, a guide for movably supporting a metal base a preselected distance from said orifice, said guide being accessible for insertion of the base therein or removal of the base therefrom during the operation of said furnace,

and means for reciprocating said base to apply successive coatings of selenium thereto.

8. Apparatus for depositing a layer of selenium upon a metal base which comprises a selenium vaporizing furnace having a narrow slot-like discharge orifice, and a pair of slotted guide members at opposite respective sides of said orifice to slidably receive and support a metal base a preselected distance from said orifice, whereby said base may be moved along the slotted portions of said guides during operation of the furnace.

9. Apparatus for depositing a layer of selenium upon a metal base which comprises a plurality of selenium vaporizing furnaces each having a narrow slot-like discharge orifice, and a guide common to all of said furnaces for passing a metal base, in succession, a preselected distance from the respective discharge orifices whereby a coating of selenium is applied to the base by the gases discharged from each furnace.

10. In the art of depositing a selenium layer of substantially uniform thickness upon at least one surface of a metal base, the steps which comprise vaporizing selenium at substantially atmospheric pressure, forming the resulting vapors into a thin ribbonlike stream in substantially unadulterated vaporized form, directing said stream of gas against a metal base while effecting relative transverse movement between said stream and said base to deposit a thin adherent coating of selenium on one surface of said base, and maintaining a protective gaseous envelope around said stream of selenium and said surface while the deposition is carried out to inhibit the formation of oxides of selenium, said envelope being formed by a gas selected from the group consisting of inert gases and reducing gases.

11. In the art of depositing a selenium layer of substantially uniform thickness upon a surface of a metal base, the steps which comprise vaporizing selenium at substantially atmospheric pressure, forming the resulting vapors into a thin unadulterated stream of gas, moving a metal base transversely through said stream to deposit an adherent selenium coating on at least one surface thereof, and surrounding said stream and said surface with a gas selected from the group consisting of inert gases and reducing gases to prevent formation of oxides of selenium.

C. SCUDDER SMITH.

#### REFERENCES CITED

The following references are of record in the file of this patent:

#### UNITED STATES PATENTS

| Number    | Name      | Date          |
|-----------|-----------|---------------|
| 2,339,613 | Becker    | Jan. 18, 1944 |
| 2,199,104 | Johnson   | Apr. 30, 1940 |
| 1,132,687 | Ryan      | Mar. 23, 1915 |
| 2,100,045 | Alexander | Nov. 23, 1937 |
| 2,103,623 | Kott      | Dec. 28, 1937 |
| 2,123,227 | Dieling   | July 12, 1938 |
| 2,334,554 | Hewlett   | Nov. 16, 1943 |
| 2,273,941 | Dorn      | Feb. 24, 1942 |

#### FOREIGN PATENTS

| Number     | Country | Date          |
|------------|---------|---------------|
| 70 805,066 | France  | Nov. 10, 1936 |